

March 24, 1936.

R. E. SCHIRMER

2,035,015

METALLIC TREATMENT OF VITREOUS MATERIALS

Original Filed Dec. 1, 1930



Fig. 2.



INVENTOR.

R. E. SCHIRMER.

BY

*James L. Dickey*

ATTORNEY.

## UNITED STATES PATENT OFFICE

2,035,015

## METALLIC TREATMENT OF VITREOUS MATERIALS

Rens E. Schirmer, New York, N. Y.

Application December 1, 1930, Serial No. 499,303  
Renewed May 22, 1935

4 Claims. (Cl. 91—70.1)

This invention relates to a method of metallizing the surfaces of vitreous materials, such as glass, porcelain, quartz, etc., to provide a metal coating thereon and in intimate and unitary contact therewith. Such a coating is not only highly desirable for certain purposes but is positively essential for the performing of certain operations or functions, among which may be mentioned the forming of sealing contacts, heat conductive purposes, increasing tensile strength, providing ornamental effects, etc. The primary object of my invention is to provide a new and improved method of producing such metallic coatings in intimate and secure contact with vitreous surfaces.

I am aware that metallic coatings have been provided on vitreous surfaces by the use of adhesives but such coatings have not been in intimate and unitary contact with the vitreous surfaces, and are quite readily removable particularly under the action of heat. I also understand that some of the rare and noble metals, such as gold and platinum, which are oxidizable only at very high temperatures, have heretofore been applied directly to vitreous surfaces but the use of such process has been extremely limited, particularly due to the high cost of these metals. My invention contemplates the use of the more common or "base" metals, such as copper, silver, nickel, etc., which oxidize relatively easily. In accordance with my invention, I first apply the metal in oxide form to the surface to be coated and so heat treat this surface that the oxide impregnates into the surface to form a physical-chemical union therewith and therebeneath. I thereafter subject this heated surface to a reducing atmosphere which reduces the exposed oxide to its metallic state in a manner leaving a pure metal coating on said surface and in intimate union with the impregnated metal in the vitreous body beneath its surface. Such an improved method of metallizing vitreous surfaces by the use of the "base" metals to provide a layer of such metal on and in intimate contact therewith comprises a further object of my invention.

In the accompanying drawing I have illustrated one simple way of carrying my invention into practice but it will be understood that the invention can be otherwise embodied and that the drawing is not to be construed as defining or limiting the scope of the invention, the claims appended hereto being relied upon for that purpose.

Referring to the figures of the drawing,

Fig. 1 illustrates the heat treatment of a coat-

ed vitreous surface in accordance with my invention;

Fig. 2 illustrates the reducing of the treated surface to provide a metallic coating thereon.

My invention particularly contemplates the coating of the surfaces of vitreous bodies with the more common and cheaper "base" metals in such manner that the metal will form an intimate and unitary contact with the bodies and render the surfaces for most purposes substantially the same as though the entire body were of metal. I have in the accompanying drawing rather diagrammatically illustrated the steps of my process and in defining the invention herein I shall briefly refer to this drawing.

Proceeding with the description of my process, I take a finely powdered oxide of the desired metal and intimately mix the same with a suitable liquid vehicle or carrier, whereby to form a paint-like paste. In employing my invention, I have most commonly used cuprous oxide intimately mixed with oil of lavender, balsam or the like. I then paint, spray, or in any other suitable manner apply a coating of the mixture to the vitreous surface to be metallized. The coating is then dried, the vehicle or oil dissipating and leaving on the vitreous surface a uniform coating of the oxide. I then introduce the coated surface into a flame or other heat treating apparatus or means, whereby its temperature is raised to the point wherein the oxide will chemically unite with the vitreous material on and beneath its surface, this usually being to a red or somewhat hotter heat.

The temperature of this heat treatment should be high enough to bring the oxide to its molten or plastic condition, whereby the oxide may be reduced to relatively pure metal in the subsequent operation which I am about to describe. The duration of this heat treatment should be sufficient to allow the chemical union to be carried out and this ordinarily takes but a few moments. Preferably directly following this treatment and without permitting the surface to cool, I quickly introduce the heated surface into a reducing atmosphere, such as hydrogen gas, whereupon the exposed oxide coating is reduced to the metallic state and is left combined in chemical union with the oxide impregnated beneath the surface of the vitreous material.

In the accompanying drawing, I indicates a tube of glass, porcelain or the like, an end portion 2 of which has been coated with cuprous oxide previously mixed with a vehicle such as oil of lavender, and which coating has thereafter been dried. This end 2 is illustrated as intro-

15

15

20

25

30

35

40

45

50

55

duced into a flame which may be an ordinary Bunsen burner or any burner which will give the required temperature, it being understood that the temperature required will vary with the 5 metal used and with the character and size of the vitreous material. After the end 2 has been sufficiently treated in the flame, it is quickly introduced into a tube 4 through which is flowing a stream of hydrogen or other gas of a reducing 10 nature, the gas escaping from this tube burning at the end 5 thereof. I have found ordinary illuminating gas very satisfactory for this purpose. The tube may be placed on a pair of rests 15 6 and is allowed to cool in the reducing atmosphere. After this cooling operation, the treated surface of the tube 1 will be found to have a coating of pure copper metal in intimate contact with the vitreous body and in chemical union with the copper impregnated thereinto. 20 The thickness of this copper coating will to a limited degree depend upon the amount of copper oxide which was originally coated upon the tube at 2. The copper surface 1 will, furthermore, be found to have substantially all the properties of 25 a solid copper tube, such as permitting soldering or fusing thereonto, a conductor of electricity, heat transmission, etc.

While I have herein more particularly referred to copper and to treatment by the use of apparatus such as illustrated in the drawing, it will be understood that any suitable metal may be used in the process and that any source of heat, such as electrical or an electrical or fuel fired furnace may be used. Furthermore, many other 35 variations thereof can be used without departing from the spirit of the invention, particularly when adapting the process to the use of automatic machine methods. It will also be understood that instead of introducing the treated tube 1 into a reducing atmosphere, the reducing atmosphere 40 may be introduced into the kiln or like apparatus in which the tube is heat treated.

Having thus described my invention, what I claim as new and desire to secure by Letters 45 Patent is:

1. A method of providing a layer of pure base metal on the surface of a vitreous body and intimately combined with the body beneath its surface, consisting of coating the surface with 50 a paint-like substance comprising an oxide of the

metal in a liquid vehicle, heat treating the coated surface at a temperature causing a portion of the coating to impregnate into and unite chemically with the body beneath its surface, and thereafter subjecting the heated surface to a reducing atmosphere to render the resulting exterior portion of the coating purely metallic and in chemical union with said coating impregnated beneath the surface. 5

2. A method of providing a layer of pure copper 10 on the surface of a vitreous body and intimately combined with the body beneath its surface, consisting of coating the surface with cuprous oxide in a liquid vehicle, subjecting the coated surface to a temperature sufficient to cause a portion 15 of the oxide to impregnate into the body beneath its surface, and reducing the resulting exterior portion of the coating to a purely metallic state by subjecting it in heated condition to a reducing atmosphere. 20

3. A method of providing a layer of pure base metal on the surface of a vitreous body and intimately combined with the body beneath its surface, consisting of coating the surface with a paste-like mixture comprising an oxide of the 25 metal in a suitable vehicle, evaporating the vehicle to dry the coating, heat treating the coated surface at a temperature causing a portion of the coating to impregnate into and unite chemically with the body beneath its surface, and 30 thereafter subjecting the coated surface in heated condition to a reducing atmosphere to render the exterior portion of the coating purely metallic and in chemical union with said coating impregnated beneath the surface. 35

4. A method of providing a layer of predetermined thickness of pure base metal on and in intimate contact with the surface of a vitreous body, consisting of mixing an oxide of the metal in a suitable liquid vehicle to form a semi-liquid 40 paste, coating the surface with the paste to a depth in accordance with the thickness of metal coating it is desired to produce, heat treating the coated surface in a flame to a temperature causing a portion of the coating to impregnate 45 into and intimately combine with the body, and thereafter subjecting the heated surface to a reducing atmosphere to render the exterior portion of the coating purely metallic.

RENS E. SCHIRMER.

50